

# UNITED STATES PATENT OFFICE.

THOMAS J. MAYALL, OF READING, MASSACHUSETTS.

## RUBBER VENEER.

SPECIFICATION forming part of Letters Patent No. 247,835, dated October 4, 1881.

Application filed May 7, 1881. (No specimens.)

*To all whom it may concern:*

Be it known that I, THOMAS J. MAYALL, of Reading, in the county of Middlesex and Commonwealth of Massachusetts, have invented a new and useful Improvement in Rubber Veneers, of which the following is a specification.

Heretofore veneer has been made of wood, sawed or cut into thin sheets from the finest and most beautiful qualities, generally too scarce and costly to make solid furniture or cabinet-work from.

The object of my invention is to provide a substitute for the veneer now used, which shall be equally ornamental and beautiful, and which will be far more durable and economical.

My invention relates, mainly, to the materials of which the veneer is made and the manner of making it; and it consists in making thin sheets of hard rubber, colored in imitation of rose-wood, mahogany, black-walnut, and other woods used for veneer and furniture and cabinet-work, and of so disposing the colors as to copy almost exactly the appearance of the grain of such woods in curls, knots, burls, branches, &c.

To make the rubber thin sheets I thoroughly mix and incorporate in a mass rubber and either of the sulphides (or sulphurets) of antimony in equal or about equal parts, by weight, and I give the desired colors to the mass by using such of the colored sulphides or sulphurets of antimony as will produce the color or combination of colors desired in the veneer. I run this compound mass out into thin sheets, and when desirable to do so back the sheets with muslin, stockinet, cotton fiber, paper, or any other suitable fabric or material; or I use the sheet rubber and sulphide (or sulphuret) of antimony compound without any backing, and in either case cure the compound by heat to the degree of hardness required for the veneer, in substantially the same manner that ordinary hard rubber is cured.

To give the outer surface of the veneer a smooth polished surface I cover it with tin-foil or other metal or substance of like smooth sur-

face, carefully laid onto the surface of the veneer so as to be in contact with every part of it, and put it under some pressure while it is in the process of curing. When it is cured the tin-foil is removed and the surface under it is found to be perfectly smooth, having a better finish than can possibly be given to wood veneer.

This veneer is hard enough to resist injury from such blows or concussions as furniture or cabinet-work is likely to receive in common use, and it is completely impervious to water and all other fluids, even the strongest acids will not affect it, and any and all foreign substance can be washed off it as readily as from a piece of porcelain, leaving no trace or injury.

I affix this veneer to the wood of furniture and cabinet-work by the use of glue in precisely the same manner that wood veneer is affixed.

To cure the rubber and sulphide (or sulphuret) of antimony compound I prefer to expose it to the action of heat at about 275° to 320° Fahrenheit for a period which may vary, according to circumstances, from about three hours to six hours.

Other proportions of rubber and sulphide (or sulphuret) of antimony may be used and cured in the manner described; but the proportions mentioned above produce the finest finished and most durable veneer.

I claim as new and my invention—

1. As a new article of manufacture, veneer made of a compound of rubber and sulphide (or sulphuret) of antimony, colored and cured to the proper hardness by heat, substantially as described.

2. As a new article of manufacture, veneer made of a compound of rubber and sulphide (or sulphuret) of antimony run into sheets and backed with cloth, stockinet, paper, or other fibrous fabric, and cured to the proper hardness by heat, substantially as described.

THOS. J. MAYALL.

Witnesses:

CHS. HOUGHTON,  
H. KENNEY, Jr.